

## UNITED STATES PATENT OFFICE

2,075,268

## SOLVENT REFINING OF LUBRICATING OIL

Louis A. Clarke, Fishkill, N. Y., assignor to The Texas Company, New York, N. Y., a corporation of Delaware

No Drawing. Application April 17, 1935, Serial No. 16,753

4 Claims. (Cl. 196—13)

This invention relates to refining hydrocarbon oil, and more particularly to refining mineral oil by solvent extraction.

The invention contemplates the treatment and refining of mineral oil with a selective solvent. It also contemplates a process of manufacturing lubricating oil wherein the lubricating oil stock is treated with a selective solvent liquid to separate it into fractions having desired characteristics, such as high viscosity index.

The invention has particular reference to the extractive treatment of mineral lubricating oil with a solvent selected from the aryl esters of halogenated fatty acids, such as halogenated acetic, propionic and butyric acids. I have discovered that the aryl esters of these halogenated fatty acids, such as benzylchloracetate and phenylethylchloracetate, are particularly suitable as solvents for the refining of mineral lubricating oil. These compounds have the following chemical structure:



The foregoing solvent liquids have been found suitable for the treatment of mineral lubricating oil stock for the production therefrom of high viscosity index lubricating oil products.

Lubricating oil fractions, such as produced from Mid-Continent crude, contain paraffinic hydrocarbon constituents as well as relatively non-paraffinic hydrocarbon constituents including naphthenic, aromatic and unsaturated hydrocarbon bodies. I have found that the paraffinic and relatively non-paraffinic constituents of lubricating oil can be separated by extractive treatment with the foregoing types of solvent liquid as, for example, benzylchloracetate.

In the application of my invention to the treatment of mineral oil for the production of a lubricating oil product, one part of the oil is mixed with from one to two parts of the solvent liquid, and this mixture is then subjected to agitation while maintained at a suitable temperature. Thereafter, the mixture, while maintained at the proper temperature, is allowed to separate into an extract and a raffinate phase. The extract phase contains the relatively non-paraffinic portion of the oil dissolved in the solvent, while the

raffinate phase comprises the undissolved paraffinic portion of the oil mixed with some of the solvent liquid.

The solvent liquid is then removed from the extract and raffinate phases by distillation, or by washing with other and more volatile solvents.

The extent to which the oil is soluble in the solvent will depend upon the nature of the particular oil undergoing treatment, as well as upon the conditions of temperature and the proportions of solvent used in making the extraction. The degree of temperature and the particular proportions of solvent to oil may be varied, depending upon the degree of extraction desired.

As a specific example, a dewaxed lubricating oil distillate obtained from Mid-Continent crude and having the tests indicated below was extracted with benzylchloracetate. The oil was extracted with about an equal volume of the solvent at a temperature of around 75° F. The mixture was separated into extract and raffinate phases, and the raffinate phase, upon removal of the solvent liquid, comprised about 76% of the original charge.

The tests on the oil before extraction, and on the resulting raffinate oil were as follows:

|                                                        | Before extraction | Raffinate oil |
|--------------------------------------------------------|-------------------|---------------|
| Gravity A. P. I. ....                                  | 21.3              | 25.8          |
| Saybolt universal viscosity in seconds at 100° F. .... | 1236              | 774           |
| Saybolt universal viscosity in seconds at 210° F. .... | 80.5              | 71.5          |
| Carbon residue percent. ....                           | .69               | .2            |
| Viscosity index. ....                                  | 51                | 77            |

In some instances, it may be of advantage to carry out the extraction in the presence of a modifying solvent liquid, such as benzol or a light petroleum fraction, such as propane or butane, for the purpose of facilitating the extraction and further controlling the extent thereof.

While esters of chloracetic acid have been specifically mentioned above, it is contemplated that the esters of other halogen substituted acids may be used. These include the esters of fluor, brom, and iodo acids as well as the di- and tri-halogen substituted acids.

The oil may be subjected to the foregoing extraction treatment, either before or after dewaxing, or subsequent to treatment with other solvents or chemicals.

The invention is not necessarily limited to the treatment of lubricating oil distillate fractions, since the solvent may be adapted to the refining

and purification of various hydrocarbon or mineral oil fractions, including naphtha, kerosene, etc., as well as residual lubricating oil fractions.

The extractive treatment of mineral oil with the foregoing solvents may be carried out in either continuous countercurrent operation, or in an intermittent batch-treating operation. Extraction may be effected in a countercurrent tower type of apparatus in which the solvent is introduced near the top of a vertical tower, while the oil to be treated is introduced near the bottom of the tower. In such case, the extract phase is removed from the bottom of the tower, while the raffinate phase is removed from the top thereof.

Obviously, many modifications and variations of the invention, as hereinbefore set forth, may be made without departing from the spirit and scope thereof, and therefore only such limitations should be imposed as are indicated in the appended claims.

I claim:

1. In the refining of mineral lubricating oil containing relatively paraffinic and relatively non-paraffinic constituents to separate therefrom a paraffinic portion of high viscosity index, the method which comprises mixing the oil with an aryl ester of a halogenated fatty acid selected from the group consisting of phenylethylchloracetate and benzylechloracetate, forming an extract phase containing non-paraffinic constituents dissolved in the solvent, and a raffinate phase comprising paraffinic oil of high viscosity index, and separating the two phases.

2. In the refining of mineral lubricating oil containing relatively paraffinic and relatively non-paraffinic constituents to separate therefrom a paraffinic portion of high viscosity index, the method which comprises mixing the oil with benzylchloracetate, forming an extract phase containing non-paraffinic constituents dissolved in the solvent, and a raffinate phase comprising paraffinic oil of high viscosity index, and separating the two phases.

3. In the refining of mineral lubricating oil containing relatively paraffinic and relatively non-paraffinic constituents to separate therefrom a paraffinic portion of high viscosity index, the method which comprises mixing the oil with phenylethylchloracetate, forming an extract phase containing non-paraffinic constituents dissolved in the solvent, and a raffinate phase comprising paraffinic oil of high viscosity index, and separating the two phases.

4. In the refining of hydrocarbon oil containing relatively paraffinic and relatively non-paraffinic constituents to separate the oil into fractions respectively rich in paraffinic and non-paraffinic constituents, the method which comprises mixing the oil with an aryl ester of a halogenated fatty acid selected from the group consisting of phenyl ethyl chloracetate and benzyl chloracetate, forming an extract phase containing non-paraffinic constituents dissolved in the solvent and a raffinate phase comprising paraffinic constituents of the oil, and separating the two phases.

LOUIS A. CLARKE.